

1

2,988,416

**PROCESS OF CREASEPROOFING LINEN FABRIC  
BY APPLYING RESIN, MERCERIZING AND RE-  
APPLYING RESIN AND PRODUCT PRODUCED  
THEREBY**

Frederick Charles Wood, Manchester, England, assignor to Tootal Broadhurst Lee Company Limited, Manchester, England, a British company

No Drawing. Filed Apr. 19, 1957, Ser. No. 653,760  
Claims priority, application Great Britain Apr. 19, 1956

11 Claims. (Cl. 8—115.6)

This invention relates to improvements in the treatment with synthetic resins of linen textile fabrics manufactured wholly or partly from flax.

In the treatment of linen textile fabrics to improve their resistance to, and recovery from, creasing by the formation of a synthetic resin inside and substantially not outside the fibres of the fabric, it has hitherto been customary to treat the fabric with resin-forming condensation products by means of a single impregnation and after resin formation to subject the fabric to a swelling, or swelling and shrinking, treatment. Thus it has been customary to treat linen fabrics, which have been treated with resin, with a swelling agent in the manner described in our U.S. Patent No. 2,158,494. The quantity of resin formed in the linen fabric when treated according to the example of U.S. Patent No. 2,158,494 is about 15%. It is necessary to iron fabrics treated in this manner after normal use and washing.

By the process of the present invention, however, there is produced a linen textile fabric having good crease-resisting properties, and moreover having such properties that a garment made of such fabric and which has been worn, washed and dried, needs only the minimum of pressing or ironing before being worn again. Linen fabrics treated according to the present invention have such smooth drying properties to a greater degree than linen fabric treated by hitherto known processes.

The condensation of formaldehyde with urea to produce a resin-forming condensation product is customarily carried out in the presence of a quantity of a solution in water of ammonia having a specific gravity of 0.88, equivalent to 8.8% by weight calculated on the weight of urea, as condensing agent. When this quantity of ammonia is used in preparing the resin-forming condensation product from formaldehyde and urea in the molecular proportion of 1.6:1, one tenth of the quantity of formaldehyde combines with the ammonia and is prevented from combining with the urea, and the equivalent proportions will be different if larger or smaller quantities of ammonia or no condensing agent, or a condensing agent other than ammonia, is used. Thus a molecular proportion of formaldehyde to urea of 1.6:1 in the presence of a quantity of a solution in water of ammonia having a specific gravity of 0.88, equivalent to 8.8% by weight calculated on the weight of urea is equivalent to a molecular proportion of  $1.6 \times 9/10:1$ , i.e. 1.44:1 where no condensing agent, or a condensing agent other than ammonia, is used. Where higher molecular proportions of formaldehyde to urea than 1.6:1 are used then the proportion of formaldehyde which is prevented from combining with the urea compared with the total quantity of formaldehyde present is less than one tenth in simple proportion. Similarly where larger or smaller quantities of ammonia than the customary quantity stated above are used, the quantity of formaldehyde which is prevented from combining with the urea varies in simple proportion. In the present invention where condensing agents which do not combine with the formaldehyde are used or greater or less quantities of ammonia are used, suitable adjustments to the molecular proportions must be made.

2

According to the present invention, a process for the production of a linen textile fabric having thermosetting synthetic resin within and substantially not between the fibers is provided in which the fabric is, in a first stage, impregnated with a low-viscosity resin-forming condensation product, which penetrates within the fibers of the fabric, formed from urea and formaldehyde in the molecular proportion of formaldehyde to urea between the limits of 1.4:1 and 2.5:1 inclusive and containing an acidic or potentially acidic catalyst, the fabric then being heated to form such resin and thereafter being subjected to a swelling, or swelling and shrinking, process as set forth in our U.S. Patent No. 2,158,494, and in which, in a second stage, the fabric is further impregnated with a low-viscosity resin-forming condensation product, which penetrates within the fibers of the fabric, formed from urea and formaldehyde in the molecular proportion of formaldehyde to urea between the limits 1.4:1 and 2.5:1 inclusive and containing an acidic or potentially acidic catalyst,

20 the fabric again being heated to form such resin without thereafter being subjected to a swelling, or swelling and shrinking, process, the amount of resin formed in the fabric as a result of the first stage impregnation and remaining in the fabric after the swelling, or swelling and shrinking, process being between the limits of 1% and 13% inclusive, the amount of resin formed in the fabric as a result of the second stage impregnation being between the limits 1% to 9% inclusive, and the total amount of resin in the fabric being between the limits of 4% and 18% inclusive, the percentage resin contents being calculated on the weight of the dry fabric before treatment and the molecular proportions of formaldehyde to urea being calculated on the basis that a quantity of a solution of ammonia in water having a specific gravity of 0.88, equivalent to 8.8% by weight calculated on the weight of urea is to be added as condensing agent, or the equivalent molecular proportion where a larger or smaller quantity of ammonia or no condensing agent or a condensing agent other than ammonia is to be used.

40 We prefer in treating line fabrics according to this invention to use molecular proportions of formaldehyde to urea in both stages of impregnation between the limits of 1.4:1 and 2.0:1 inclusive calculated on the basis that a quantity of a solution of ammonia in water having a specific gravity of 0.88, equivalent to 8.8% by weight calculated on the weight of urea is to be added as condensing agent, or the equivalent molecular proportion where a larger or smaller quantity of ammonia or no condensing agent or a condensing agent other than ammonia is to be used. We prefer to treat such fabrics so that the quantity of resin formed in the fabric as a result of the first stage impregnation and remaining in the fabric after the swelling, or swelling and shrinking, treatment is between the limits 3 and 8% inclusive, and so that the quantity of resin formed in the fabric as a result of the second stage impregnation is between the limits 3 and 6% inclusive and so that the total quantity of resin in the fabric is between the limits of 6 and 14% inclusive.

All percentages of resin contents given hereinafter are calculated on the weight of the dry fabric before treatment with resin-forming condensation product.

In carrying out the present invention it is preferred to use such an amount of resin-forming condensation product in the first stage that the amount of resin remaining in the fabric after the swelling, or swelling and shrinking, process is smaller than is normally used to produce crease-resisting properties. The formation in the fabric in the second stage of a suitable amount of synthetic resin to bring about the production of good dry crease-resisting properties results in the production, in addition, of good smooth drying properties. Indeed, it is possible by treating the

linen fabric with resin-forming condensation product in two stages, of which only the first stage includes a subsequent swelling, or swelling and shrinking, process, to obtain better dry crease-resisting properties than are obtained by the same quantity of resin insolubilised in a single stage which includes such subsequent swelling, or swelling and shrinking, process. For example, the formation in a linen fabric of 7½% of synthetic resin from formaldehyde and urea in the molecular proportion of 1.6:1, and reduction of this to 4½% by a swelling, or swelling and shrinking, process, gives a fabric having poor dry crease-resisting properties, but after the formation in the fabric of sufficient synthetic resin from formaldehyde and urea in the molecular proportion of 1.6:1 in the second stage to give a total resin content of 10-12%, a better dry crease-resisting property is developed which is moreover better than that of a fabric treated so as to contain 10-12% of resin using formaldehyde and urea in the molecular proportion of 1.6:1 after a single impregnation followed by a swelling, or swelling and shrinking, process. Moreover the fabric treated in two stages has in addition good smooth drying properties.

The swelling, or swelling and shrinking, process is carried out with any of the swelling agents, including caustic soda of mercerizing strength, and in the manner described, in our prior specification No. 2,158,494. In the preferred embodiment of this invention where the amount of resin formed in the fabric during the first stage of the process of this invention is smaller than the amount normally used in a one stage process, the swelling, or swelling and shrinking, of the fabric takes place more rapidly than normally. During this process some of the synthetic resin which has been insolubilised by heating is removed, and this must be taken into account in adjusting the treatment so that the required quantity of resin remains in the fabric after the first stage of the treatment and in the final fabric. The quantity of resin should be adjusted so that the final fabric possesses simultaneously good crease-resisting and good smooth drying properties, and good physical properties of tensile strength and resistance to wear. Furthermore the higher the molecular proportion of formaldehyde to urea used in forming the resin in both stages of impregnation, the smaller the total amount of resin which it is preferred to form on the fabric because the resistance to wear of the finished fabric may be seriously affected. Thus when using molecular proportions of formaldehyde to urea greater than 2:1 in both stages of impregnation we prefer that the total amount of resin formed in the fabric should not exceed 12% or better should not exceed 8%.

Conversely the lower the molecular proportion of formaldehyde to urea used in forming the resin in both stages of impregnation, the greater the total amount of resin which it is preferred to form in the fabric. Thus when using molecular proportions of formaldehyde to urea less than 1.6:1 in both stages of impregnation calculated on the basis that a quantity of a solution of ammonia in water having a specific gravity of 0.88, equivalent to 8.8% by weight calculated on the weight of urea is to be added as condensing agent, or the equivalent molecular proportion where a larger or smaller quantity of ammonia or no condensing agent or a condensing agent other than ammonia is to be used, we prefer that the total amount of resin formed on the fabric should be at least 7%, or better at least 9%.

We prefer, according to this invention, to treat linen fabrics which have not been mercerized before resin treatment. It has been found that if treatment of the fabric, including mercerization, prior to the first stage resin treatment is kept to a minimum, better all round physical properties, for example crease-resisting properties and resistance to wear are obtained.

Linen fabrics which have not been mercerized and which have received the first resin treatment and then

been subjected to a swelling, or swelling and shrinking, process, may then be dyed. In this way a better colour yield is frequently obtained in comparison with the same fabric which has been dyed before resin treatment, thereby reducing dyestuff costs, and since the fabrics are not subsequently subjected to a severe caustic alkali treatment the range of dyestuffs which may be used is increased.

The treatment of linen fabrics according to this invention may include treatment with a lubricating agent for example as described in our British application No. 31150/55, filed November 1, 1955. Suitable lubricating agents are a methylol derivative of a condensation product of a higher fatty acid chloride with a polyethylene polyamine sold under the trade name "Sapamine WP," or a dimethylol stearyl melamine sold under the trade name "Phobotex FT."

The resin may be formed in either or both stages of the treatment in atmospheres containing more than 50% of superheated steam, for example as described in our prior U.S. specification No. 3,29,774, filed August 22, 1955, now U.S. Patent 2,859,136.

The catalyst present in the impregnating mixtures may be a weak acid, such as tartaric acid, or a potential acid, such as ammonium dihydrogen phosphate, which liberates acid on heating in the presence of the impregnating mixture. Alternatively we may use the acid salt of a polybasic acid having a dissociation constant in water of not less than  $10^{-6}$  with a metal of which a less acid salt with the same polybasic acid is precipitated before said acid salt on concentration and/or on heating the solution, for example sodium dihydrogen phosphate and magnesium sulphate, as described in our co-pending U.S. application No. 581,508, filed April 30, 1956. When steam is used to form the resin such catalyst is preferably one which does not develop sufficient acidity during the low temperature drying to form more than a very small proportion of the total resin formed on the fabric to ensure that as much as possible of the resin is formed in the presence of superheated steam.

The low viscosity resin forming condensation products formed from urea and formaldehyde which are used in the present invention, may be alkylated to form alkylated methylol ureas and then used to impregnate linen textile fabrics according to the present invention.

By "linen textile fabric" we mean fabric containing at least 25% by weight of flax. The present invention therefore includes the treatment of mixture fabrics containing at least 25% by weight of flax and also containing other cellulosic fibre such as cotton or regenerated cellulose or non-cellulosic fibres such as nylon.

The invention will be more clearly understood by reference to the following examples which are purely illustrative.

#### EXAMPLE 1

2 gallons of aqueous formaldehyde solution containing 40 grammes of formaldehyde per 100 ccs. of solution, 10 lb. of urea (molecular proportion of formaldehyde to urea 1.6:1) and 405 ccs. of ammonia (specific gravity 0.88) were allowed to stand at room temperature until the mixture reached equilibrium in density and viscosity. This mixture was diluted until the density was 19° Tw. (approximately 5½ gallons).

To 5½ gallons of this mixture was added 14 oz. of ammonium dihydrogen phosphate dissolved in a little water, 4 oz. of a mixture of sodium cetyl and oleyl sulphates mixed with water and the mixture was further diluted with water to about 10 gallons. The density of this mixture (Mixture A) was 10° Tw.

A portion of Mixture A was further diluted with water until its density was 7° Tw., Mixture B.

#### First stage impregnation

An absorbent fabric made of 100% flax and weigh-

ing 200 gms. per square metre and having in the loom state 25 combed tow warp threads per inch and 32 combed tow weft threads per inch, of 30 and 25 lea respectively, previously well scoured and bleached was impregnated with Mixture A and passed between the bowls of a mangle adjusted so as to leave about 65% of liquor on the fabric, dried on a stenter and then heated at 300° F. for three minutes. The fabric was then passed through an aqueous solution containing as wetting agent 1/4% of an alkali salt of a sulphonated fatty alcohol and 1/4% of soda ash at 80° C. The fabric was then squeezed and whilst still wet run into a bath of 65° Tw. caustic soda. It was then lightly squeezed so as to leave caustic soda on the fabric and was allowed to stand without tension either in warp or weft for 10 minutes during which time it was allowed to shrink in both directions. The fabric was then washed with water over a mercerizing stenter until neutral and dried on steam heated cylinders. At this stage the fabric contained 4.7% of resin.

#### Second stage impregnation

The treated fabric was then impregnated with Mixture B, dried and heated in the same way as in the first stage impregnation. It was then washed at 80° C. for 30 seconds in 1/2% soda ash, washed in water and mangled and passed through a bath containing 1% of a mixture of 3 parts of stearin to 1 of borax, and dried on steam heated cylinders. It was then damped with water and cold and calendered and finished on a controlled compressive shrinkage machine.

By the second stage impregnation the fabric was treated with a further 4.3% of resin and the total resin content of the finished fabric was 9.0%.

The finished fabric showed excellent dry crease-resistance and dresses made of the fabric could be worn, washed, squeezed free of excess water and when dried by hanging on a clothes hanger they could be worn without being ironed. The fabric had these properties to a greater degree than a similar fabric treated so as to contain 9.0% of resin by a single impregnation followed by a swelling and shrinkage treatment.

nation was used for all samples. The variations used are shown in the table given below.

Each sample was then tested to obtain its Smooth Drying Index (S.D.I.), Ring Wear (R.W.) figures.

The S.D.I. figures were obtained by use of the apparatus described in our co-pending U.S. application No. 628,902, filed December 17, 1956, now Patent 2,909,921 and consisting of (1) a crease maker, (2) a drying cabinet, and (3) a crease gauge.

Specimen strips of the fabric under test are cut in both warp and weft directions. These are wetted-out, squeezed through a small domestic mangle, and inserted in the crease maker in order to form a sharp double crease. The specimen is next dried for half an hour and during drying the crease inserted in the wet fabric diminishes. The S.D.I. figure is obtained from the extent of this recovery and it indicates the ability of the fabric to recover from creases formed during normal domestic washing.

The extent of this recovery is measured by placing the dried sample in the cabinet of the crease gauge and the angle of the residual crease is measured from observation of the shadow cast by the crease when illuminated by a directional light source. The smaller the figure obtained in this test the better is the fabric's property of needing little or no ironing after washing.

The R.W. figures were obtained by use of the Ring Wear Machine described in the Textile Recorder Year Book 1942-3 page H36. In this machine a standard

wool fabric is placed over the face of one disc and the test fabric is placed over the face of another disc of similar size. The two discs are placed face to face so that the wool fabric and the test fabric are in friction contact, one disc being offset from the other, so that the circumference of each disc passes through the approximate centre of the other. To test the abrasion resistance of the test fabric both discs are set to revolve until the test fabric breaks down under friction with the wool fabric. The number of revolutions required to reach this point is taken as a measure of the resistance to wear.

All the samples treated and tested showed good resistance to creasing in the dry state.

| Ratio of formaldehyde to urea         |           | Resin, Percent |           |       | Strength of impregnating mixture, °Tw. |           | Physical Properties of finished fabric |                          |
|---------------------------------------|-----------|----------------|-----------|-------|----------------------------------------|-----------|----------------------------------------|--------------------------|
| 1st Stage                             | 2nd Stage | 1st Stage      | 2nd Stage | Total | 1st Stage                              | 2nd Stage | S.D.I.                                 | R.W.(No. of revolutions) |
| 1.4.....                              | 1.4       | 13             | 4         | 17    | 28                                     | 6 1/2     | 11                                     | 800                      |
|                                       |           | 8              | 6         | 14    | 17                                     | 10        | 11                                     | 930                      |
|                                       |           | 7              | 4         | 11    | 15                                     | 6 1/2     | 12                                     | 1,400                    |
|                                       |           | 5              | 4         | 9     | 10 1/2                                 | 6 1/2     | 12 1/2                                 | 1,470                    |
|                                       |           | 2              | 6         | 8     | 4                                      | 10        | 12 1/2                                 | 1,200                    |
|                                       |           | 11             | 4         | 15    | 23                                     | 6 1/2     | 10 1/2                                 | 900                      |
| 1.4.....                              | 1.8       | 7              | 4         | 11    | 15                                     | 6 1/2     | 13                                     | 950                      |
|                                       |           | 5              | 3         | 10    | 15                                     | 5         | 14                                     | 1,200                    |
|                                       |           | 2              | 4         | 6     | 4                                      | 6 1/2     | 12 1/2                                 | 1,100                    |
|                                       |           | 8              | 2         | 10    | 17                                     | 3         | 13                                     | 950                      |
|                                       |           | 7              | 2         | 9     | 15                                     | 3         | 11                                     | 1,050                    |
|                                       |           | 2              | 3         | 5     | 4                                      | 5         | 12                                     | 1,000                    |
| Ratios between 2.0 and 2.5 inclusive. | 1.4       | 8              | 3         | 11    | 15                                     | 5         | 12 1/2                                 | 850                      |
|                                       |           | 4              | 3         | 7     | 7                                      | 5         | 13                                     | 1,200                    |
|                                       |           | 1              | 6         | 7     | 2                                      | 10        | 13                                     | 930                      |
|                                       |           | 8              | 2         | 10    | 15                                     | 3         | 14 1/2                                 | 1,100                    |
|                                       |           | 4              | 2         | 6     | 7                                      | 3         | 12                                     | 1,050                    |
|                                       |           | 1              | 4         | 5     | 2                                      | 6 1/2     | 13 1/2                                 | 800                      |
| Ratios between 2.0 and 2.5.           | 1.8       | 7              | 1         | 8     | 13                                     | 1 1/2     | 14                                     | 950                      |
|                                       |           | 4              | 1         | 5     | 7                                      | 5         | 12                                     | 1,100                    |
|                                       |           | 1              | 3         | 4     | 2                                      | 5         | 14 1/2                                 | 1,100                    |
|                                       |           | 7              | 2         | 9     | 13                                     | 3         | 13                                     | 1,000                    |
|                                       |           | 4              | 2         | 6     | 7                                      | 3         | 12                                     | 1,200                    |
|                                       |           | 1              | 3         | 4     | 2                                      | 5         | 14                                     | 1,000                    |
| Ratios between 2.0 and 2.5.           | 2.5       | 7              | 1         | 8     | 13                                     | 1 1/2     | 14                                     | 950                      |
|                                       |           | 4              | 1         | 5     | 7                                      | 5         | 12                                     | 1,100                    |
|                                       |           | 1              | 3         | 4     | 2                                      | 5         | 14 1/2                                 | 1,100                    |
|                                       |           | 7              | 2         | 9     | 13                                     | 3         | 13                                     | 1,000                    |
|                                       |           | 4              | 2         | 6     | 7                                      | 3         | 12                                     | 1,200                    |
|                                       |           | 1              | 3         | 4     | 2                                      | 5         | 14                                     | 1,000                    |

#### EXAMPLE 2

Different samples of a fabric as in Example 1 were treated as described in Example 1, but suitable adjustments were made in the quantities of urea and formaldehyde used and in the extent of dilution of the partially condensed mixture, to form on the samples different quantities of resin. Mangle adjustment so as to leave about 65% of liquor on the fabric after impreg-

I claim:

1. A process for improving the crease resisting and smooth drying properties of a linen textile fabric containing at least 25% by weight of flax comprising the steps of impregnating said fabric with a low viscosity resin-forming solution comprising formaldehyde, urea and a catalyst for the reaction of said formaldehyde and said urea, the molecular proportion of said formaldehyde to

said urea being from 1.4:1 to 2.5:1, applying heat to the impregnated fabric to insolubilize the urea-formaldehyde reaction product within the fibres of the fabric, mercerizing said fabric with a mercerizing agent under conditions which permit the fabric to shrink, said fabric having a urea-formaldehyde resin content of from 1 to 13% inclusive based on the weight of the dry fabric prior to treatment, further impregnating said treated fabric with said low viscosity resin-forming solution, heating said impregnated fabric to insolubilize additional urea-formaldehyde resin within the fibres of said fabric, said additional resin being present in an amount of from 1 to 9% based upon the weight of the dry fabric, the total weight of the resin on the fabric being within the range of 4 to 18% inclusive, said fabric being held in a flat position after each of said impregnating steps while said resin is being insolubilized thereon.

2. Process as claimed in claim 1 in which the quantity of resin formed in the fabric as a result of the first step impregnation and remaining in the fabric after being mercerized by the mercerizing agent is between the limits of 3% and 8% inclusive.

3. Process as claimed in claim 1 in which the quantity of resin formed in the fabric as a result of the second step impregnation is between the limits of 3% and 6% inclusive.

4. Process as claimed in claim 1 in which the total quantity of resin in the fabric is between the limits of 6% and 14% inclusive.

5. Process as claimed in claim 1 in which the linen fabric has been scoured and bleached but not mercerized before the first impregnation step.

6. Process as claimed in claim 1 in which the heating to form the resin after one of said impregnation steps is effected in an atmosphere containing more than 50% of superheated steam.

7. Process as claimed in claim 1 in which the heating to form the resin after both impregnation steps is effected in an atmosphere containing more than 50% of superheated steam.

8. The process as defined in claim 1 wherein said molecular proportions of formaldehyde to urea are between the limits of 1.4:1 and 2.0:1 inclusive.

9. The process as defined in claim 1 wherein said fabric is made of 100% flax.

10. A process for improving the crease resisting and smooth drying properties of a linen textile fabric containing at least 25% by weight of flax comprising the steps of impregnating said fabric with a low viscosity resin-forming aqueous solution comprising formaldehyde, urea and a catalyst for the reaction of said formaldehyde and said urea, the molecular proportion of said formaldehyde to said urea being from 1.4:1 to 2.0:1, applying heat to the impregnated fabric to insolubilize the urea-formaldehyde reaction product within the fibres of the fabric, mercerizing said fabric with a mercerizing agent under conditions which permit the fabric to shrink, 15 said fabric having a urea-formaldehyde resin content of from 3 to 8% inclusive based on the weight of the dry fabric prior to treatment, further impregnating said treated fabric with said low viscosity resin-forming solution, heating said impregnated fabric to insolubilize additional urea-formaldehyde resin, said additional resin being within the range of 3 to 6% based upon the weight of the dry fabric, the total weight of the resin on the fabric being within the range of 6 to 14% inclusive, said fabric being held in a flat position after each of said 20 impregnating steps while said resin is being insolubilized thereon.

11. The crease-resistant and smooth-drying linen textile fabric produced by the process defined in claim 1.

30 **References Cited in the file of this patent**  
**UNITED STATES PATENTS**

|           |         |       |              |
|-----------|---------|-------|--------------|
| 1,734,516 | Foulds  | ----- | Nov. 5, 1929 |
| 2,158,494 | Corteen | ----- | May 16, 1939 |
| 2,859,136 | Marsh   | ----- | Nov. 4, 1958 |

40 **FOREIGN PATENTS**

|         |               |       |               |
|---------|---------------|-------|---------------|
| 437,361 | Great Britain | ----- | Oct. 25, 1935 |
| 607,582 | Great Britain | ----- | Sept. 1, 1948 |

**OTHER REFERENCES**  
 Marsh, John T.: An Introduction to Textile Finishing, 1948, pages 390, 402.